

# UNITED STATES PATENT OFFICE.

HENRY LAVERS, OF CAMBERWELL, ALFRED HENRY PIPER LOWRY, OF PRAHRAN, AND HENRY HOWARD GREENWAY, OF MELBOURNE, VICTORIA, AUSTRALIA, ASSIGNORS, BY MESNE ASSIGNMENTS, TO MINERALS SEPARATION AMERICAN SYNDICATE (1913) LIMITEL, OF LONDON, ENGLAND.

## CONCENTRATION OF SULFID ORES.

1,208,171.

Specification of Letters Patent. Patented Dec. 12, 1916.

No Drawing.

Application filed March 14, 1914. Serial No. 824,765.

To all whom it may concern:

Be it known that we, HENRY LAVERS, a subject of the King of England, residing at Camberwell, Victoria, Australia, ALFRED 5 HENRY PIPER LOWRY, a subject of the King of England, and residing at Lynzala, High street, Prahran, State of Victoria, Australia, and HENRY HOWARD GREENWAY, a subject of the King of England, residing at Mel- 10 bourne, Victoria, Australia, have invented certain new and useful Improvements in the Concentration of Sulfid Ores, of which the following is a specification.

This invention relates to certain improvements in the concentration of sulfid ores, and refers more especially to the concentration of mixed zinc and lead sulfid ores, that is to say ores containing a mixture of galena and blende with gangue. In this specification 15 the term "ores" is intended to include concentrates, tailings, slimes, and other products containing metallic sulfids.

This invention relates to the concentration of sulfid ores by flotation separation, and 20 more especially to froth flotation separation, in which a froth of sulfids is floated to the surface consequent upon the aeration or agitation of the ores in the presence of a suitable frothing agent (such as an essential oil—for instance—eucalyptus oil).

Hitherto froth flotation separation of the mixed sulfids from the gangue has generally been conducted with the addition of acid to the circuit water. With certain ores— 25 known as calcitic ores—containing carbonates the consumption of acid has in some instances largely added to the cost of treatment. This applies especially to slimes, as the acid consuming substances (such as calcite, &c.) are mostly found with the finely divided slimes. An alkaline medium or circuit water has been adopted in some cases, and, under certain conditions, for the differential or preferential flotation separation 30 of certain sulfids from other sulfids, but so far as we are aware, a flotation separation of mixed sulfids generally from the gangue has not been effected with the employment in solution in the pulp of an alkaline selectivity-modifying agent. It has 35 previously been proposed to effect the concentration of copper ores by the agitation froth process by agitating the ore sus-

pended in water with a minute quantity of an aromatic hydroxy compound to beat in 55 air and form a froth, at the same time adding to the circuit solution a small proportion of an alkali to facilitate the solution of the aromatic hydroxy compound employed as a frothing agent. 60

We have discovered that if a finely pulverized ore is submitted to flotation separation with agitation and aeration and with a suitable frothing agent (such as an essential oil, for instance eucalyptus oil) in water 65 containing in solution an alkaline substance, such as carbonate of soda; a froth of the metallic sulfids will rise to the surface and may be separated from the gangue which sinks. This separation is preferably effected at a temperature of from 120° to 70 130° F. We have also found that the addition of an organic frothing agent (such as eucalyptus oil) is not always necessary, as the presence of the said alkaline substance in the solution in some cases is sufficient to insure the formation of a mineral bearing froth. 75

The question as to whether in the treatment of any particular ore in a certain circuit water the addition of an organic frothing agent is necessary can be determined by a simple laboratory test. 80

If desired the resultant products may be retreated with or without the addition of 85 fresh quantities of the substances referred to.

As an example of the application of this process we may mention certain experiments which have been conducted by us:— 90

A. One pound of slimes assaying 14.4% lead, and 14.6% zinc, was submitted to flotation separation with agitation and aeration in 4 lbs. of water containing in solution carbonate of soda equivalent to 22.4 lbs. 95 per ton of slimes treated, to which was also added eucalyptus oil equivalent to 0.6 lbs. per ton of slimes. The charge was thoroughly aerated by being agitated in such a way as to disseminate air through the mixture. On bringing the mixture to rest, a froth of mixed concentrates was obtained assaying 26% lead, and 29.8% zinc, leaving a residue assaying 3.3% lead, and 2.2% zinc. 100

B. A parcel containing one ton of slimes 105 from Broken Hill assaying 11% lead and

15.6% zinc, was thoroughly aerated by being agitated in about four (4) tons of water containing an amount of soda ash equivalent to 35 lbs. per ton of ore treated, and 5 eucalyptus oil equivalent to three-quarters ( $\frac{3}{4}$ ) of a lb. per ton of ore treated at a temperature of from 125° to 130° F. A froth of mixed sulfids was obtained assaying 18.5% lead and 27.4% zinc, being a recovery 10 of 90% lead and 94% zinc. These float concentrates were retreated with small additions of eucalyptus oil and soda ash to the circuit water equivalent to 0.1 lbs. and 4 lbs. respectively per ton of ore treated 15 while the temperature was maintained at about 125° to 130° F., when a froth of mixed sulfids was obtained assaying 22.4% lead and 35.8% zinc, being a recovery of 84.3% lead and 90% zinc.

20 C. Two lbs. of Broken Hill slimes were mixed with 7 lbs. water at 130° F., and soda ash equal to 22.4 lbs. per ton of the slimes. The mixture was then thoroughly aerated by being agitated, with the result that a 25 mixed concentrate assaying 29.5% lead, 35.2% zinc, 25.0 ozs. per ton silver was produced, giving recoveries of 90.0% lead, 92.7% zinc, and 91.5% silver. In this test no frothing agent other than soda ash was 30 added.

D. Two lbs. of Queensland copper ore tarnished by weathering and unsuitable for ordinary flotation treatment assaying 2.9% copper (of which 0.5% copper was oxidized) 35 6.5 dwts. per ton gold were mixed with 7 lbs. water at 70° F. containing soda ash equal to 33.6 lbs. per ton of the ore and a mixture of about equal proportions of eucalyptus oil and mineral oil equivalent to 40 2 lbs. per ton of ore. The whole was then thoroughly aerated by being agitated with the result that a froth of mixed sulfids was obtained assaying 11.3% copper, 26.1 dwts. gold, being a recovery of 74.4% copper, 45 76.7% gold.

The concentrates obtained by this invention are found to be in a most suitable condition for preferential flotation separation of one of the sulfids from the other sulfids 50 by one of the known methods, more especially one employing an alkaline separating medium. Though it has been found that the above method is especially applicable to the treatment of slimes, it is not confined to the 55 treatment of that class of ore, but is applicable to coarser material also.

This method of treatment is especially applicable to cases where by reason of the state of the ore due to oxidation by exposure 60 or weathering (such as accumulated dump slimes and tarnished ores), the use of acid is inadvisable, and neutral circuit water is unsuitable.

The alkaline substances most suitable for 65 addition to the circuit water are the carbon-

ates of the alkaline metals, but other alkalis may be used. We prefer in most cases the crude sodium carbonate or soda ash. The amount of alkaline substance added to the circuit water should in all cases be sufficient to produce slight alkalinity in the mixture of ore and water when submitted to the well known phenolphthalein test. Any of the known frothing agents may be used in conjunction with the alkaline circuit water, 70 but in cases where the alkali and the frothing agent react upon one another (such as with carbonate of soda and oleic acid) the latter must be added in very small quantities to avoid the formation of an undue 80 amount of soaps which tend to form an indiscriminate froth of sulfids and gangue. We therefore prefer to use a frothing agent other than a fatty acid.

In the following claims the terms "substantially all the floatable metalliferous minerals" and "substantially all the floatable zinc and lead" are intended to mean such a recovery of metalliferous mineral or of zinc and lead together as is practically obtainable in a procedure which aims to float all the metalliferous mineral as differentiated from preferential selection of one metalliferous mineral from another.

What we claim as our invention and desire to secure by Letters Patent is:—

1. A process of concentrating ores containing mixed metalliferous minerals which consists in agitating and aerating a pulp of such an ore, such pulp containing in solution an alkaline selectivity-modifying agent, so as to obtain a froth of concentrates of substantially all the floatable metalliferous minerals while the gangue sinks, said solution being alkaline during separation of the 100 minerals, and separating the froth, whereby the metalliferous minerals are separated from the gangue.

2. A process of concentrating ores containing mixed metalliferous minerals which consists in agitating and aerating a pulp of such an ore, such pulp containing in solution an alkaline selectivity-modifying agent and also containing a small proportion of a frothing agent, so as to obtain a froth of concentrates of substantially all the floatable metalliferous minerals while the gangue sinks, said solution being alkaline during separation of the minerals, and separating the froth, whereby the metalliferous 115 minerals are separated from the gangue.

3. A process of concentrating ores containing mixed metalliferous minerals which consists in agitating and aerating a pulp of such an ore, such pulp containing in solution a carbonate of an alkaline metal, so as to obtain a froth of concentrates of substantially all the floatable metalliferous minerals while the gangue sinks, said solution being alkaline during separation of the 125 130 minerals.

minerals, and separating the froth, whereby the metalliferous minerals are separated from the gangue.

4. A process of concentrating ores containing mixed metalliferous minerals which consists in agitating and aerating a pulp of such an ore, such pulp containing in solution a carbonate of an alkaline metal and also containing a small proportion of a frothing agent, so as to obtain a froth of concentrates of substantially all the floatable metalliferous minerals while the gangue sinks, said solution being alkaline during separation of the minerals, and separating the froth, whereby the metalliferous minerals are separated from the gangue.

5. A process of concentrating ores containing mixed metalliferous minerals which consists in agitating and aerating a pulp of such an ore, such pulp containing sodium carbonate in solution so as to obtain a froth of concentrates of substantially all the floatable metalliferous minerals while the gangue sinks, said solution being alkaline during separation of the minerals, and separating the froth, whereby the metalliferous minerals are separated from the gangue.

6. A process of concentrating ores containing mixed metalliferous minerals which consists in agitating and aerating a pulp of such an ore, such pulp containing sodium carbonate in solution and also containing a small proportion of a frothing agent, so as to obtain a froth of concentrates of substantially all the floatable metalliferous minerals while the gangue sinks, said solution being alkaline during separation of the minerals, and separating the froth, whereby the metalliferous minerals are separated from the gangue.

7. A process of concentrating zinc-lead ores which consists in agitating and aerating a pulp of such an ore, such pulp containing in solution an alkaline selectivity-modifying agent, so as to obtain a froth of concentrates containing substantially all the floatable zinc and lead while the gangue sinks, said solution being alkaline during the separation of the minerals, and separating the froth, whereby the zinc and lead are separated from the gangue.

8. A process of concentrating zinc-lead ores which consists in agitating and aerating a pulp of such an ore, such pulp containing in solution an alkaline selectivity-modifying agent and also containing a small proportion of a frothing agent, so as to obtain a froth of concentrates containing substantially all the floatable zinc and lead while the gangue sinks, said solution being alkaline during separation of the minerals, and

separating the froth, whereby the zinc and lead are separated from the gangue.

9. A process of concentrating zinc-lead ores which consists in agitating and aerating a pulp of such an ore, such pulp containing in solution a carbonate of an alkaline metal, so as to obtain a froth of concentrates containing substantially all the floatable zinc and lead while the gangue sinks, said solution being alkaline during separation of the minerals, and separating the froth, whereby the zinc and lead are separated from the gangue.

10. A process of concentrating zinc-lead ores which consists in agitating and aerating the pulp of such an ore, such pulp containing in solution a carbonate of an alkaline metal and also containing a small proportion of a frothing agent, so as to obtain a froth of concentrates containing substantially all the floatable zinc and lead while the gangue sinks, said solution being alkaline during separation of the minerals, and separating the froth, whereby the zinc and lead are separated from the gangue.

11. A process of concentrating zinc-lead ores which consists in agitating and aerating a pulp of such an ore, such pulp containing sodium carbonate in solution, so as to obtain a froth of concentrates containing substantially all the floatable zinc and lead while the gangue sinks, said solution being alkaline during separation of the minerals, and separating the froth, whereby the zinc and lead are separated from the gangue.

12. A process of concentrating zinc-lead ores which consists in agitating and aerating a pulp of such an ore, such pulp containing sodium carbonate in solution and also containing a small proportion of a frothing agent, so as to obtain a froth of concentrates containing substantially all the floatable zinc and lead while the gangue sinks, said solution being alkaline during separation of the minerals, and separating the froth, whereby the zinc and lead are separated from the gangue.

In testimony whereof we have signed our names to the specification in the presence of two subscribing witnesses.

HENRY LAVERS.

ALFRED HENRY PIPER LOWRY.

HENRY HOWARD GREENWAY.

Witnesses to signatures of Henry Lavers and Alfred Henry Piper Lowry:

CHARLES V. COLLISON,

HAWLY COBEY.

Witnesses to signature of Henry Howard Greenway:

HAROLD CHARLES HANKINS,  
WILLIAM JAMES WALTON.